

## UNITED STATES PATENT OFFICE

2,099,350

## PYROLYSIS OF HYDROCARBONS

Wesley C. Stoesser, Midland, Mich., assignor to  
The Dow Chemical Company, Midland, Mich.,  
a corporation of Michigan

No Drawing. Application May 17, 1935,  
Serial No. 22,105

5 Claims. (CL 260—170)

This invention relates to improvements in processes for pyrolyzing hydrocarbons, and in particular to such processes which involve the pyrolysis of aromatic hydrocarbons, for example, 5 benzene.

One of the difficulties commonly associated with processes in which hydrocarbons are heated, either in gas or liquid phase, at high temperatures is the formation of carbon on the heating surfaces. Such carbon formation results in a loss of materials in process, while the carbon deposits so formed interfere with the transfer of heat and frequently cause interruptions of the process for removing carbon accumulations 15 which obstruct the apparatus.

In apparatus of the type used for pyrolyzing or cracking hydrocarbons iron or steel is the usual material of construction wherever it can be employed without detriment. It is known, 20 however, that at the temperatures used in various cracking processes, e. g. 500° to 900° C., iron promotes the formation of solid carbon, apparently acting as a catalyst for breaking down the hydrocarbon molecules to elementary carbon. Various expedients have been proposed for 25 avoiding the effects of the aforesaid catalytic action of iron in contact with hydrocarbons at cracking temperatures. For instance, it has been proposed to use special steels of high chromium content, but such steels are more costly than ordinary carbon steels, and in a large installation their use adds greatly to the capital cost and increases correspondingly the cost of the product. It is desirable to make possible and practicable the use of usual carbon steels in the 30 construction of apparatus for the pyrolysis of hydrocarbons.

Particularly in connection with the pyrolysis of benzene and other aromatic hydrocarbons for 35 the formation of diphenyl and related diaryl compounds it has been found that, when the pyrolysis is carried out in iron apparatus, much carbon is formed, which deposits on the walls of the apparatus, sometimes in hard compact form, at 40 others in loose form, depending upon variations in operating conditions. These carbon deposits greatly interfere with the smooth and continuous operation of the process, so much so that it has generally been regarded as impracticable to 45 use tubular apparatus of wrought iron or carbon steel for pyrolyzing benzene hydrocarbons in the usual temperature range of about 650° to 850° C., because the tubes rapidly become filled and stopped with carbon. It has therefore been proposed to employ special chromium steels for the 50

apparatus, or to provide special coatings or linings on ordinary steel which inhibit or reduce the formation of carbon, or to introduce along with the pyrolysis gases or vapors a foreign substance which has the effect of counteracting the formation of carbon. 5

I have now found that the substantial prevention of carbon formation in the pyrolysis of hydrocarbons, generally, and particularly benzene hydrocarbons, when carried out in apparatus of iron or carbon steel, can be attained by much simpler means than those hitherto used. The invention is based upon my discovery that a preliminary treatment of the iron surfaces of the pyrolyzing apparatus with ammonia serves to 15 suppress the catalytic action of iron in causing formation of carbon in the apparatus subsequently when hydrocarbons are heated to a pyrolyzing temperature therein. 10

It is among the objects of the invention to 20 provide a method of pyrolyzing hydrocarbons in ordinary iron or steel apparatus wherein the formation of carbon is greatly reduced or even substantially prevented, whereby the process can be carried on continuously for long periods of time 25 without interruption due to carbon accumulation. Another object is to provide a method of treating such iron apparatus for pyrolysis of hydrocarbons, particularly benzene hydrocarbons, so that carbon formation is practically inhibited therein during such pyrolysis. Another 30 object is to enable the use of wrought iron or common mild steels as structural material of apparatus for carrying out the aforementioned pyrolytic reactions. Other objects will appear 35 from the following specification in which the invention is fully described and particularly pointed out in the claims. 30

For purpose of illustration the invention will be described with particular reference to the 40 pyrolysis of benzene and benzene hydrocarbons for the production of diphenyl and related diaryl compounds, but in its broad scope the invention is applicable to processes for the pyrolysis of hydrocarbons in general, especially in gas 45 or vapor phase, such as in the cracking of petroleum hydrocarbons for the production of motor fuel or of gaseous olefines, and the like. 50

During a series of experiments in the pyrolysis of benzene vapors at a temperature in the range 50 of 650° to 850° C., in which the vapors were passed through heated tubes of wrought iron or low carbon steel, it was found that within a few hours at most the tubes would become practically blocked with carbon. This result occurred ir- 55

respective of the purity of the benzene, or of the rate of vapor flow, the carbon formation of course being the more rapid the higher the temperature. This situation indicated the practical impossibility of using ordinary iron or steel tubes in a commercial apparatus for making diphenyl and diaryl compounds by pyrolyzing benzene hydrocarbons, in which process the operation would have to be practically continuous over a considerable period of time in order to be commercially economical. However, I found that, if such tubes were subjected to the action of ammonia at a moderately elevated temperature for a short time prior to employing them for the pyrolysis of benzene, the latter process could then be carried out in the tubular apparatus uninterruptedly for periods of several days, even weeks, without any substantial formation of carbon.

The treatment with ammonia may easily be carried out *in situ* with the apparatus completely assembled for use in the pyrolytic process. The furnace section of the apparatus in which cracking is to be carried out is simply heated so that the cracking tubes, or the equivalent thereof, are heated to a temperature approximately in the range of 300° to 600° C., and ammonia is passed through the apparatus for a short time, e. g. from about 1/2 to 2 hours, but not necessarily exceeding a few hours at most. For example, at a temperature of around 500° C., a period of from 30 minutes to 1 hour is sufficient for the ammonia treatment. At lower temperatures a somewhat longer time may be required to give the best results. After such preliminary treatment with ammonia the apparatus may be heated to the regular operating temperature and the hydrocarbon vapors passed therethrough, the pyrolyzing process then being continued indefinitely without substantial deposition of carbon, whereas without such ammonia treatment the tubes would be blocked with carbon within a few hours at most.

The effect of the aforesaid ammonia treatment in causing suppression of carbon formation in iron apparatus is not completely understood. An X-ray examination has shown that the ammonia treatment produces a thin film of iron nitride on the exposed surface of the iron. However, subsequent exposure of such nitride coating to hydrocarbon vapors for a short time at the pyrolyzing temperature results in the disappearance of the iron nitride film, at least to the extent that it is no longer detectable by X-ray test. Nevertheless, the disappearance of the nitride film does not affect the ability of the iron surface to resist or prevent the formation and deposition of carbon thereon, in view of the fact that such a surface has been employed continuously for many days in the pyrolysis of benzene without formation of carbon taking place thereon. Apparently the action of ammonia on the iron surface renders it passive with respect to the normal property of iron to catalyze carbon formation under the conditions existing in pyrolysis reactions.

As a specific example of the practice of the invention, benzene was vaporized at the rate of 2 cubic centimeters per minute and the vapors were passed through a standard 1 inch iron pipe 53 inches long heated in a furnace over a length of 47 inches, so that the maximum temperature at about the middle of the pipe was 760°-790° C. Under these conditions the percentage conversion of benzene to diphenyl and higher diaryls was approximately 8 per cent. In 11.5 hours the pipe was completely stopped with carbon. The pipe was removed and another piece of the same length

inserted in the furnace, and ammonia gas was passed through the pipe for 1/2 hour. Thereafter benzene vapors were passed through the pipe at the same rate as before, and at an average maximum temperature of 737° C. continuously for 89.5 hours, giving a conversion of 9.23 per cent, at the end of which time no perceptible deposit of carbon had formed in the pipe. The product of the pyrolysis consisted of 86.7 per cent of diphenyl, and 13.3 per cent of higher boiling compounds.

In other experiments conducted similarly in iron pipes at temperatures varying from about 700° to 760° C. maximum, and at varying rates of vapor flow corresponding to the vaporization of from 2 to 11 cubic centimeters of benzene per minute, the pipes were stopped with carbon in from 3 to 5 hours. When similar iron pipes were given a preliminary treatment with ammonia at about 400° to 500° C. for about 1 hour, and then used to pyrolyze benzene under similar conditions of vapor flow and temperature they were run as long as 200 hours continuously without material formation of carbon.

By preventing carbon formation, the invention has the further advantage that a higher conversion of benzene to diphenyl is obtained, other conditions remaining the same. In fact, as shown in the foregoing example, a higher conversion can be obtained at a somewhat lower temperature. The invention therefore not only overcomes the mechanical and operating difficulties previously experienced, thereby making possible by simpler means than hitherto the commercial adaptation of iron apparatus in the pyrolysis of benzene and other hydrocarbons, but it also results in an increased yield of product and materially raises the efficiency of the process.

When treating the iron tubes, or other ferrous apparatus, with ammonia in accordance with the invention, it is convenient, but not necessary, to maintain a slight gas pressure, e. g. 5 to 10 pounds gauge, in the apparatus. The ammonia treatment may be carried out at any temperature suitable for nitridizing iron, e. g. between about 300° and 700° C., preferably between about 450° and 550° C.

Similarly, ferrous reactors used for the pyrolysis of other hydrocarbons, such as petroleum and fractions thereof, and aliphatic or aromatic hydrocarbons generally, may be given a preliminary treatment with ammonia to suppress the formation of carbon therein subsequently during the pyrolysis of the hydrocarbons. The treatment may be conveniently carried out *in situ* with the apparatus already set up for operation, to coat the interior walls, at least initially, with a film of iron nitride, or the parts thereof may be separately treated with ammonia in any suitable way and later assembled for use in the process.

Other modes of applying the principle of my invention may be employed instead of those explained, change being made as regards the method herein disclosed, provided the step or steps stated by any of the following claims or the equivalent of such stated step or steps be employed.

I therefore particularly point out and distinctly claim as my invention:

1. In a method of pyrolyzing hydrocarbons in apparatus constructed of iron or steel, the improvement which consists in preventing or reducing the formation of carbon by passing the hydrocarbon vapors at a pyrolyzing temperature through such apparatus of iron or carbon steel,

the walls of which exposed to contact with the vapors have been previously subjected to the action of ammonia at a nitridizing temperature for a time sufficient to form a nitride coating thereon.

5. 2. In a method of pyrolyzing benzene hydrocarbons in apparatus constructed of iron or steel, the improvement which consists in preventing or reducing the formation of carbon by passing the benzene hydrocarbon vapors at a pyrolyzing temperature through such apparatus of iron or carbon steel, the walls of which exposed to contact with the vapors have been previously subjected to the action of ammonia at a nitridizing temperature for a time sufficient to form a nitride coating thereon.

10. 3. In a method of pyrolyzing benzene hydrocarbons in apparatus constructed of iron or steel, the improvement which consists in preventing or 15 reducing the formation of carbon by passing the benzene hydrocarbon vapors at a pyrolyzing temperature through such apparatus of iron or carbon steel, the walls of which exposed to contact with the vapors have been previously subjected to the action of ammonia at a temperature between about 450° and 550° C. for a time sufficient 20 to form a nitride coating thereon.

20. 4. In a method of pyrolyzing benzene hydrocarbons in apparatus constructed of iron or steel, the improvement which consists in preventing or 25 reducing the formation of carbon by passing the benzene hydrocarbon vapors at a pyrolyzing temperature through such apparatus of iron or carbon steel, the walls of which exposed to contact with the vapors have been previously subjected to the action of ammonia at a temperature between about 450° and 550° C. for a period of from about one-half hour to about two hours.

tween about 300° and about 700° C. for a time sufficient to form a nitride coating thereon.

5. 4. In a method of pyrolyzing benzene hydrocarbons in apparatus constructed of iron or steel, the improvement which consists in preventing or 5 reducing the formation of carbon by passing the benzene hydrocarbon vapors at a pyrolyzing temperature through such apparatus of iron or carbon steel, the walls of which exposed to contact with the vapors have been previously subjected to the action of ammonia at a temperature between about 450° and 550° C. for a time sufficient to form a nitride coating thereon.

10. 5. In a method of pyrolyzing benzene hydrocarbons in apparatus constructed of iron or steel, 15 the improvement which consists in preventing or reducing the formation of carbon by passing the benzene hydrocarbon vapors at a pyrolyzing temperature through such apparatus of iron or carbon steel, the walls of which exposed to contact 20 with the vapors have been previously subjected to the action of ammonia at a temperature between about 450° and 550° C. for a period of from about one-half hour to about two hours.

WESLEY C. STOESSER. 25